

March 10, 1936.

W. BROWN

2,033,814

COMPOSITE METAL ARTICLE

Filed May 27, 1929

Fig. 1.



Fig. 2.



INVENTOR

Walter Brown

BY *Whittmore Hubbard*  
*Whittmore & Belknap*

ATTORNEYS

## UNITED STATES PATENT OFFICE

2,033,814

## COMPOSITE METAL ARTICLE

Walter Brown, Toledo, Ohio

Application May 27, 1929, Serial No. 366,468

13 Claims. (Cl. 251—167)

The invention relates to the manufacture of composite metal articles composed of two different metals or alloys integrally and continuously bonded together. More particularly the invention relates to certain articles of manufacture requiring different properties in different portions thereof, thus making the use of two different alloys desirable for the manufacture of the same. For example, a valve seat bushing for oil wells can be constructed in accordance with my invention thereby producing an article having a long life under the conditions which it meets in every day use.

In accordance with my invention the outer shell of the article is made of steel or other tough alloy while the inner surface is composed of a cobalt-chromium alloy of the type generally known by the name "Stellite". This alloy has the property of extreme hardness and resistance to abrasion and heretofore has been used mainly for cutting tools.

The inner alloy must be integrally bonded to the outer tube and it is therefore preferable to utilize the process outlined in my co-pending application (Patent No. 1,923,075) filed on even date herewith. This process briefly described consists in placing the desired amount of the solid alloy within a tube of steel or other tough alloy and after closing the ends thereof subjecting the same to a temperature sufficient to melt the alloy but not the outer tube. The tube is then rotated at a speed such that the molten alloy forms a pool at the bottom of the tube and washes the sides of the tube removing foreign matter therefrom which might otherwise interfere with the formation of a proper bond. After sufficient washing action the tube is cooled down while the rotation continues until finally the alloy congeals and forms a solid ring uniformly spaced from the axis of rotation and integrally and continuously bonded to the outer metal. The alloy is thus centrifugally cast to the inner surface of the outer tube. With certain metals and alloys it is desirable to increase the speed of rotation after the initial washing action so that the metal is evenly distributed around the tube at the time when solidification occurs.

In the drawing,

Figure 1 is an axial section through an oil well bushing;

Figure 2 is a cross section thereof.

The oil well bushing comprises an outer ring 10 formed of steel or other tough alloy having an annular rib 11 on the periphery thereof. Integrally and continuously joined thereto is the

inner ring 12 formed of a hard, wear-resisting alloy preferably comprising chromium and a metal of the class consisting of cobalt and nickel. The inner ring is of uniform diameter and has the beveled edge 13 at one or both ends thereof forming the seat for the valve.

Another composition for the inner ring is as follows:

|            | Approximate percentage |
|------------|------------------------|
| Cobalt     | 50                     |
| Chromium   | 32                     |
| Tungsten   | 16                     |
| Molybdenum | 2                      |

The above alloys have a fusing point of approximately 2350 to 2400 degrees F., whereas the melting point of ordinary steel is approximately 2800 degrees F. or above.

My invention also contemplates articles other than the oil well bushing above described. Thus, there are many other devices wherein an outer tube of a relatively tough alloy may be advantageously associated with an integrally bonded inner lining of a metal or alloy having a relatively high fusing point. Another example of my invention is a steel or other alloy tube having an inner lining of bronze. A tube of this character may be used for bearings and is superior to an all bronze bearing bushing because the latter has a different coefficient of expansion than the steel, whereas in my improved bushing the coefficient of expansion is substantially the same as steel because the steel constitutes the major part of the article. In carrying out my invention it is essential that the high fusing inner metal be integrally and continuously bonded to the outer material. By this it is meant that the lining has characteristics resulting from the fact that it has been solidified from the molten condition simultaneously over the entire surface. In view of the fact that the melting temperature of the inner alloy is relatively high, extreme care must be exercised to prevent such oxidation of the metal as would prevent the formation of the proper bond. One process adapted for the manufacture of the articles herein described and claimed is set forth in my Patent No. 1,923,075.

What I claim as my invention is:

1. A valve seat bushing comprising an outer tube of steel and a centrifugally cast inner tube integrally and continuously bonded thereto composed of a hard wear-resisting non-ferrous alloy containing chromium and a metal of the class consisting of cobalt and nickel.

2. A valve seat bushing comprising an outer metallic tube and a centrifugally cast inner tube integrally and continuously bonded thereto composed of a hard wear-resisting non-ferrous alloy containing chromium and a metal of the class consisting of cobalt and nickel, said outer tube having an annular rib extending radially outward from the outer surface thereof, and said inner tube having a bevel edge forming a valve seat.

3. A valve seat bushing comprising an outer metallic ring having an annular rib extending radially outward from the periphery thereof and a centrifugally cast inner lining integrally and continuously bonded thereto having approximately the following composition:

|             | Per cent |
|-------------|----------|
| Cobalt      | 50       |
| Chromium    | 32       |
| 20 Tungsten | 16       |
| Molybdenum  | 2        |

4. As an article of manufacture, an outer metallic tube, an inner metallic lining integrally and continuously bonded thereto, the inner lining comprising a metal having a melting point over 1000° F. and the outer member being a preformed tube of a metal having a melting point substantially higher than the melting point of the inner lining.

5. As an article of manufacture, a preformed outer tube and a centrifugally cast metallic inner lining continuously bonded thereto, said lining being of a metal having a melting point above 1000° F. and said outer tube being of a metal having a melting point substantially above the melting point of said inner metal.

6. A valve seat bushing comprising an outer steel tube and a centrifugally cast inner tube integrally and continuously bonded thereto composed of a non-ferrous alloy containing chromium, tungsten and a metal of the class consisting of cobalt and nickel, said steel tube having an annular rib extending radially outward from the outer surface thereof and said inner tube having a bevel edge forming a valve seat.

7. As an article of manufacture, a preformed outer tube and a centrifugally cast metallic inner lining, said lining being of a metal having a melting point above 1000° F. and having a metallic

structure characteristic of centrifugally cast metal, said outer tube being of a metal having a melting point substantially above the melting point of said inner metal, said inner metal being continuously bonded to said outer metal.

8. A valve seat bushing comprising an outer metallic tube and a centrifugally cast inner tube integrally and continuously bonded thereto composed of a hard wear-resisting non-ferrous alloy comprising chromium and a metal of the class consisting of cobalt and nickel.

9. As an article of manufacture, a preformed outer tube and a centrifugally cast metallic inner lining continuously bonded thereto, said lining being of a hard wear-resisting metal having a melting point above 1000° F. and said outer tube being of steel having a melting point substantially above the melting point of said inner metal.

10. As an article of manufacture, a preformed outer steel tube and a centrifugally cast bronze inner lining continuously bonded thereto, said bronze lining having a melting point above 1000° F. and said steel outer tube having a melting point substantially above the melting point of said bronze lining.

11. As an article of manufacture, a preformed metallic tube, a centrifugally cast metallic layer integrally and continuously bonded thereto, the centrifugally cast metallic layer having a melting point above 1000° F. and the preformed metallic tube having a melting point substantially above the melting point of said centrifugally cast metallic layer.

12. As an article of manufacture, a preformed metallic tube, a centrifugally cast metallic layer integrally and continuously bonded thereto, the centrifugally cast metallic layer being of a hard wear-resisting metal having a melting point above 1000° F. and said preformed tube being of steel having a melting point substantially above the melting point of said hard wear-resisting metal.

13. As an article of manufacture, a preformed metallic tube, a centrifugally cast metallic layer integrally and continuously bonded thereto, the centrifugally cast layer being of bronze having a melting point above 1000° F. and said preformed tube being of steel having a melting point substantially above the melting point of said bronze.

WALTER BROWN. 50